

May 16, 1961

A. G. CHERREAU ET AL

2,983,998

BIMETAL ELEMENTS

Filed Dec. 2, 1957

2 Sheets-Sheet 1

*Fig. 1.*



Inventors

André G. Cherreau  
André R. M. Girard  
Albert J. P. Villachon  
by Stevens, Davis, Miller & Mathen  
their attorneys

May 16, 1961

A. G. CHERREAU ET AL

2,983,998

BIMETAL ELEMENTS

Filed Dec. 2, 1957

2 Sheets-Sheet 2



Fig: 2



Fig: 3

Patentees  
André G. Cherreau  
André R. M. Girard  
Albert J. P. Villachage  
by Stevens, Davis, Miller & Kauff  
their attorneys

## BIMETAL ELEMENTS

André G. Cherreau and André R. M. Girard, Imphy, Nièvre, and Albert J. P. Villachon, Paris, France, assignors to Societe Metallurgique d'Imphy (Societe Anonyme), Paris, France, a company of France

Filed Dec. 2, 1957, Ser. No. 700,130

Claims priority, application France Aug. 8, 1949

3 Claims. (Cl. 29—195.5)

This application is a continuation-in-part of our co-pending application Ser. No. 474,577, filed Dec. 10, 1954, now abandoned, which was already a continuation-in-part application of our original application Ser. No. 174,525, filed July 18, 1950, now abandoned.

This invention relates to bimetal elements.

Bi-metal strips or blades which are used in numerous forms of apparatus having a thermal action such as thermostats, regulators, circuit breakers and the like comprise, as is known, two alloys: one having a very high coefficient of expansion and the other having a low coefficient of expansion. When the strips, suitably assembled, are raised to a certain temperature, the difference in the expansion of the alloys causes the strip to curve which produces a desired action. This curvature can be expressed by the value of a "specific deflection," namely the amount of displacement of one end of a straight bimetal strip fixed at the other end, the strip having an effective length of 100 mms. and a thickness of 1 mm., produced by an increase of temperature of 1° C. The properties of the bimetal strip can also be defined by Villarceau's coefficient:

$$V = \frac{3}{2}(\alpha_2 - \alpha_1)$$

$\alpha_1$  and  $\alpha_2$  being the coefficients of expansion of the two components of the strip.

The components having a high expansion of known bimetal strips are very numerous. Thus, for example, the following metals have been successively used, viz: iron, having a coefficient of expansion at ordinary temperatures of the order of  $12.10^{-6}$ ; copper, having a coefficient of expansion of the order of  $18$  to  $20.10^{-6}$ ; nickel, having a coefficient of expansion of the order of  $16.10^{-6}$ ; iron-nickel-chromium alloy, having about 23% of nickel and a low chromium content of 2.5%, the coefficient of expansion of which is of the order of  $20$  to  $22.10^{-6}$ ; another ferro-nickel containing about 15 to 20% of nickel and 5 to 9% of manganese, and having a coefficient of expansion amounting to as much as  $22$  to  $23.10^{-6}$ .

Special alloys have also been recently used containing more than 70% of manganese, the remainder being nickel and copper in variable proportions; these alloys have the advantage of coefficients of expansion which can be as high as  $27.10^{-6}$ . In all these cases, however, the component of low coefficient of expansion has been selected from binary iron-nickel alloys. An alloy frequently used is a ferro-nickel containing 36% of nickel and commonly known by the name of Invar (registered trademark owned by the applicant company), whose coefficient of expansion at room-temperature is the lowest. This alloy exhibits, however, an anomaly in its expansion consisting in an extremely rapid increase in the coefficient of expansion, starting from 175° C. As the high expansion elements above-mentioned or actually known which can be associated with Invar do not show a similar anomaly either with regard to temperature or to intensity, it fol-

lows that the bi-metal strips produced up to the present with Invar lose much of their sensitivity above 175° C.

The invention will be explained by reference to the drawings:

5 Figure 1 is a diagram showing the deflection of bi-metal strips as a function of the temperature.

Figs. 2 and 3 are curves taken with a Chevenard differential dilatometer showing the relative expansion of an element having a high and an element having a low coefficient of expansion, each with respect to a standard element.

The above effect is illustrated by curves 1', 2', 3' of Fig. 1 on which the temperature in degrees centigrade are shown as abscissae and the specific deflections of the bimetal strips in millimetres are shown as ordinates. The three bimetal strips corresponding to the curves 1', 2', 3' have as the low expansion component a ferro-nickel containing 36% of nickel and as the high expansion component either a ferro-nickel chromium alloy containing 23%

20 nickel and 2.5% of chromium (curve 1') or a manganese-copper-nickel alloy containing 74% of manganese, 15% of copper and 10% of nickel (curve 2') or pure nickel (curve 3'). It will be seen that the best of three bimetal strips, namely that producing the curve 2' still shows a decrease in sensitivity above 200° C. Moreover, their deflection is linear, i.e. approximately proportional to the increase of temperature, but only between the room-temperature and 160° C. (curve 1'), 150° C. (curve 2') or 170° C. (curve 3') approximately; this temperature limit is still too low for many industrial applications.

25 The foregoing observations have led the applicants to investigate the possibility of finding means for making bimetal elements with a high and linear deflection up to temperatures which are as high as possible, which is very important for numerous practical applications, and particularly for electric circuit breakers.

30 In order to find the solution of this problem, it did not suffice to know the properties of a certain number of metals and alloys, on the one hand with a low coefficient of expansion and on the other hand with a high coefficient of expansion, and to compare their diagrams of thermal expansion.

35 As will be seen later, this theoretical study leads to erroneous conclusions, and only practical work and tests have enabled the object to be attained.

40 Binary iron-nickel alloys other than Invar have a comparable anomaly leading to a similar disadvantage in the case of bimetal strips. This anomaly disappears at high temperatures with an increase in the nickel content, but simultaneously therewith the coefficient of expansion of the iron-nickel increases very rapidly, which leads to a reduction in the sensitivity of the bimetal strips in substantial proportions.

45 For these various reasons, the conclusion has been reached that Invar and the other known iron-nickel binary alloys should not be used for the low expansion component, and a different metal should be sought.

It is known that ternary alloys comprising 16 to 20% 50 of Co and 27 to 30% of Ni—the remainder being substantially iron—have a coefficient of expansion which although bigger than that of Invar is still very small, and this within a fairly high temperature range.

55 It has however been thought up to the present time that the bi-metallic strips in which these alloys are employed as an element of low coefficient of expansion could not have a deflection proportional to the temperature between 0° and 400° C. because the thermal expansion of these alloys is irregular in this range of temperature.

60 This irregularity is shown by a study of their expansion by the differential method, which has become usual since accurate and convenient differential dilatometers

have become available, such for example as the well-known Chévenard instruments, which automatically record the difference between the expansion of the substance studied and that of a standard having a uniform expansion free from any anomalies, in the vicinity of that of the sample under study, and sufficiently creep resistant at the temperatures considered; such standards may be constituted for example by pure molybdenum for the samples with low coefficient of expansion and, for samples with a high coefficient of expansion by an alloy of 85 to 88% nickel, 8 to 10% chromium and 2 to 3% tungsten, known by the name of Pyros.

The diagram of differential expansion reproduced in Fig. 2 relates to an alloy with a high coefficient of expansion comprising 14.65% copper and 10.81% nickel, the remainder being essentially manganese. The temperature is plotted as abscissae and the differences between the expansion of the sample and that of the standard of Pyros alloy, the well-known law of expansion of which is perfectly regular, are plotted as ordinates; the diagram shows that the expansion of this Mn—Cu—Ni alloy is large and perfectly uniform.

But the expansion diagram of Fig. 3, which shows in a similar manner the difference between the coefficient of expansion of an Fe—Ni—Co alloy with 27.8% nickel and 18.25% cobalt, usable as an alloy with a low coefficient of expansion, referred to that of a standard of molybdenum free from any expansion anomalies, shows on the contrary that the expansion of the Fe—Ni—Co alloy exhibits not only the anomaly corresponding to the point of disappearance of magnetism or Curie point, situated between 400° and 450° C., but also shows between the ambient temperature and 400° a further anomaly of expansion, less pronounced but still perfectly clear; the expansion of the sample is first greater, and then when the temperature rises still further, smaller than that of the standard of molybdenum.

These anomalies of expansion exist for all the Fe—Ni—Co alloys, the Curie point of which is situated above 350° C., and in particular for those which contain 27 to 30% of nickel and 16 to 20% of cobalt.

Since the differences in expansion between the two constituents of the bi-metallic strip do not follow a linear law as a function of the temperature, the bi-metallic strip formed by the association of this Fe—Ni—Co alloy of low coefficient of expansion with an alloy of high coefficient of expansion and free from any expansion anomalies, such as for example the Mn—Cu—Ni alloy which has just been mentioned, should not in theory have a deflection proportional to the temperature, or linear, over the whole range from 0° to 400° C.

Following these scientific indications, in order to form a bi-metallic strip of high sensitivity and with a deflection proportional to the temperature up to 400° C., it would thus be necessary to reject the use of the Fe—Ni—Co alloys of low coefficient of expansion of the composition indicated, in spite of their advantages. This is perhaps the reason why it has never been proposed to employ them to constitute the low-expansion element of a bi-metallic strip, associated with an alloy of high coefficient of expansion selected from the group comprising the alloys Mn—Cu—Ni with 13 to 20% of copper and 8 to 12% of nickel, and the Fe—Ni—Mn alloys with about 14 to 20% of nickel and 5 to 9% of manganese which are attractive because of their large and uniform expansion.

It has thus been unexpected and surprising to find, during the course of research tests and check tests that, contrary to what might have been theoretically expected, the irregularities of the differences between the coefficients of expansion of the two elements in the temperature range from 0° to 400° C. do not appear in the utilisation of the bi-metallic strip, for reasons which are not yet entirely clear, but which might be connected, at least in part, to phenomena of relaxation or accommodation.

Thus the applicants have obtained, for the first time, bi-metallic strips of high sensitivity having a deflection practically proportional to the difference in temperature up to 400° C., and which are entirely satisfactory for all practical requirements, and this constitutes a substantial technical progress: in fact, the specific deflection of these new bi-metallic strips is 1.8 to 2.8 times as great as that of the best bi-metallic strips known up to the present time, which have a linear deflection up to 400° C.

In conclusion, the applicants have discovered that the result envisaged in accordance with the invention, that is to say the manufacture of bi-metallic elements of high sensitivity and having a linear deflection up to a temperature reaching, or even exceeding 400° C., has been obtained by the combination of two elements constituted respectively by the alloys specified below.

Alloy with a small coefficient of expansion:

10 Nickel ----- 27 to 30% and preferably 28 to 29%.  
15 Cobalt ----- 16 to 20% and preferably 16.5 to 18.5%.  
20 Iron ----- Substantially the remainder.

Alloy with a high coefficient of expansion:

25 Copper ----- 13 to 20%.  
Nickel ----- 8 to 12%.  
Manganese ----- Substantially the remainder.  
or  
30 Nickel ----- 14 to 20%.  
Manganese ----- 5 to 9%.  
Iron ----- Substantially the remainder.

These three alloys may, of course, include in addition the usual contents of secondary elements, such as silicon (or manganese in the case of the first) etc., of impurities such as sulphur, phosphorus, etc.

The bi-metallic members obtained by the association of these alloys are free from anomalies likely to hinder their operation or their use, up to temperatures of the order of 400° C.

The element with a high coefficient of expansion has preferably a composition which falls within the following limits:

45 Copper ----- approximately 15%.  
Nickel ----- approximately 10%.  
Manganese ----- Substantially the remainder.  
or  
50 Nickel ----- approximately 15%.  
Manganese ----- approximately 7%.  
Iron ----- Substantially the remainder.

The same reservations apply as in the previous case with respect to the presence of secondary elements or impurities.

55 The electrical resistivities of the bi-metallic strips in accordance with the invention may vary within fairly wide limits, as shown by the examples below:

60 (1) The bi-metallic strip, of which the low-expansion element is an Fe—Ni—Co alloy of 27% nickel and 18% cobalt, and the high-expansion element is an Fe—Ni—Mn alloy with 15% nickel and 7% manganese has a specific deflection of 0.115 mm. per degree centigrade, and a resistivity of 50 microhms per sq. cm. per cm.

65 Curve 1 on the Fig. 1 shows that the deflection of such a bi-metallic strip having a length of 10 cm. and a thickness of 1 mm., is practically proportional to the temperature up to above 400° C.

70 (2) The bi-metallic strip, of which the low-expansion element is an Fe—Ni—Co alloy with 27% nickel and 18% cobalt, and the high-expansion element is an Mn—Cu—Ni alloy with 15% copper and 10% nickel has a specific deflection of 0.170 mm. per degree centigrade and a resistivity of 70 microhms per sq. cm. per cm.

75 Curve 2 on the Fig. 1 shows that the deflection of such a bi-metallic strip having a length of 10 cm. and

a thickness of 1 mm., is practically proportional to the temperature up to 400° C.

The deflection of these bi-metallic strips is much greater than that of the bi-metallic strip of which the low-expansion element would be of an Fe—Ni—Co alloy of the same composition as in these two examples, and the high-expansion element were of pure nickel.

Without departing from the scope of the invention, known means may be employed for modifying the electrical resistance of the bi-metallic strips described, for example by interposing between the two basic elements a sheet of an alloy of high or low resistivity; for example, in the second case, a sheet of nickel, or of iron, or of brass, or a coating of brazing-solder, etc.

What we claim is:

1. A bimetal element of high sensitivity, capable of linear deflection with reference to a temperature between 0 and 400° C., comprising a first elongated part having a low coefficient of expansion and formed from an alloy consisting of iron, nickel and cobalt, the alloy comprising 27 to 30% of nickel and 16 to 20% of cobalt, the remainder being substantially iron, a second elongated part longitudinally and closely united to the first part and made of an alloy having a high coefficient of expansion selected from the group consisting of manganese-copper-nickel alloys with 13 to 20% of copper and 8 to

10

5

12% of nickel, the remainder being substantially manganese, and iron-nickel-manganese alloys comprising 14 to 20% of nickel and 5 to 9% of manganese the remainder being substantially iron.

2. A bimetal element according to claim 1, wherein the part having a high coefficient of expansion is of manganese-nickel-copper alloy comprising approximately 75% of manganese, 15% of copper and 10% of nickel.

3. A bimetal element according to claim 1, wherein the part having a high coefficient of expansion is of iron-nickel-manganese alloy comprising approximately 15% of nickel and 7% of manganese.

15

#### References Cited in the file of this patent

#### UNITED STATES PATENTS

|           |       |               |
|-----------|-------|---------------|
| 1,843,903 | Scott | Feb. 2, 1932  |
| 1,902,589 | Scott | Mar. 21, 1933 |
| 1,939,085 | Scott | Dec. 12, 1933 |
| 1,987,714 | Scott | Jan. 15, 1935 |
| 2,062,335 | Scott | Dec. 1, 1936  |
| 2,062,836 | Scott | Dec. 1, 1936  |
| 2,234,748 | Dean  | Mar. 11, 1941 |
| 2,349,577 | Dean  | May 23, 1944  |
| 2,403,895 | Alban | July 16, 1946 |